

[54] METHOD FOR THE PRODUCTION OF A MATTED TRANSPARENT PAPER AND THE PRODUCT THEREOF

[75] Inventors: Noritoshi Watanabe, Nishinomiya; Masato Nakamura, Toyonaka; Seigoro Fujita, Amagasaki, all of Japan

[73] Assignee: Kanzaki Paper Manufacturing Co., Ltd., Tokyo, Japan

[\*] Notice: The portion of the term of this patent subsequent to Sep. 4, 1996, has been disclaimed.

[21] Appl. No.: 957,834

[22] Filed: Nov. 6, 1978

#### Related U.S. Application Data

[63] Continuation of Ser. No. 723,137, Sep. 14, 1976.

#### Foreign Application Priority Data

Sep. 18, 1975 [JP] Japan 50-113176

[51] Int. Cl.<sup>3</sup> D21H 5/12

[52] U.S. Cl. 162/146

[58] Field of Search 162/146, 157 R, 187, 162/206, 362, 117, 141, 143, 150, 151, 109; 427/121; 29/121.8; 264/284

[56]

#### References Cited

##### U.S. PATENT DOCUMENTS

|           |         |                       |           |
|-----------|---------|-----------------------|-----------|
| 1,992,996 | 3/1935  | Dodge .....           | 162/187   |
| 3,235,443 | 2/1966  | Greenman et al. ..... | 162/187   |
| 3,412,479 | 11/1968 | Markovic .....        | 29/121.8  |
| 3,486,970 | 12/1969 | Troemel et al. .....  | 162/157 R |
| 3,674,621 | 7/1972  | Miyamoto et al. ..... | 162/146   |
| 3,892,887 | 7/1975  | Shibata et al. .....  | 427/121   |
| 4,015,043 | 3/1977  | Watanabe et al. ..... | 162/146   |

#### FOREIGN PATENT DOCUMENTS

44-5326 of 1969 Japan

#### OTHER PUBLICATIONS

Tappi Data Sheet, "Freeness Scale Interconversion", Corr. 1945.

Primary Examiner—Peter Chin

Attorney, Agent, or Firm—Armstrong, Nikaido, Marmelstein & Kubovcik

[57]

#### ABSTRACT

A matted transparent paper is obtained by moistening a paper prepared from relatively lightly beaten pulp and then subjecting the moistened paper to a calendering treatment with the use of a heated embossing metal roll having a finely engraved surface with sharp reliefs.

8 Claims, 14 Drawing Figures

FIG. 1



FIG. 2



FIG. 3



FIG. 4





FIG. 5



FIG. 6



FIG. 7



FIG. 8

*FIG. 9*



*FIG. 10*



*FIG. 11*



*FIG. 12*





FIG. 13



FIG. 14

**METHOD FOR THE PRODUCTION OF A  
MATTED TRANSPARENT PAPER AND THE  
PRODUCT THEREOF**

This is a continuation of application Ser. No. 723,137, filed Sept. 14, 1976.

**BACKGROUND OF THE INVENTION**

This invention relates to the production of a matted transparent paper which is improved in writability, paper strength, dimensional stability and secondary processability.

A tracing paper, a master copy paper and a paper for plotter are usually required to have a uniform transparency and a good writability with a pencil or an aqueous ink. Those papers have been generally prepared by subjecting papers made of heavily beaten pulp having a Canadian Standard Freeness (hereinafter referred to as CSF) of within the range of 50 to 100 cc or less to a treatment with heat and pressure under a high moisture content with the use of a calender. However, the heavy beating of pulp promotes an injury and a hydration of pulp fibers and the papers made of such heavily beaten pulp have various practical disadvantages such as a low paper strength for example tear resistance and a low dimensional stability to moisture. In addition, a paper sheet treated by for example a heated super calender for the purpose of obtaining a high transparency has a very smooth surface, and accordingly is inferior in a writability.

Japanese Patent Publication No. 5,326 of 1969 discloses a process for making a transparent paper in which natural pulp, synthetic pulp or a mixture thereof is formed into a paper and then heat and pressure are applied to the resultant paper under the condition of the moisture content of the paper being 10 to 30% with the use of a flat plate or a roll having such an uneven surface that its surface roughness,  $H_{max}$ , which is defined in Japanese Industrial Standard (hereinafter referred to as JIS) BO601-1955; is within the range of 2 to 20 microns, and a height of the fine relief peak on the surface is within the range of 0.2 to 1 micron. This technique has improved a writability of paper which has never been satisfactorily obtained in the conventional calendering techniques by forming finely uneven structures on the surface of the paper with use of a particular calender system provided with the uneven surface roll. The paper thus obtained has an improved writability, but this technique still depends on the conventional heavily beaten pulp for obtaining a transparency which is one of the other important required characteristics. Since this technique depends on a limited method such as a sand blast method for forming the finely uneven structures on the surface of the roll, the processed surface of the roll is limited to the extremely fine structures having the patterns peculiar to the sand blast method. Therefore, a satisfactory and uniform transparency cannot be obtained when the paper is made of pulp having a CSF larger than 100 cc though it can be obtained in the case of the paper being composed of heavily beaten pulp. The above technique uses, practically, the pulp whose beating degree is within the range of 90 to 95SR according to a Schopper-Riegler method described in JIS P8121. This value of beating degree corresponds to a CSF of one figure value which shows that the pulp is beaten to an extremely high ex-

tent. The disadvantages due to such a heavy beating have been already described hereinbefore.

As described above, according to the prior arts, it has never been possible to obtain a tracing paper or a master copy paper superior in a uniformity of transparency, paper strength, writability, dimensional stability and secondary processability with the use of such an ordinarily beaten pulp that is used in making a general wood free paper.

According to the invention, the above described problems in the prior arts can be solved. This invention is based on a discovery which is against the heretofore accepted theory that a heavy beating is required for obtaining a sufficient transparency of sheet. This invention is characterized by that a paper is prepared from ordinarily or lightly beaten pulp and then heat and pressure are applied to the resultant paper with aid of a special embossing metal roll whereby the problem of decrease in transparency inherent in the use of such lightly beaten pulp is solved.

An object of the invention is to provide a matted paper which has a uniform transparency and is improved in writability, paper strength, dimensional stability and secondary processability.

Other objects and advantages of the invention will become apparent from the following descriptions.

**SUMMARY OF THE INVENTION**

According to the invention, a paper is prepared from an aqueous suspension of pulp having a CSF larger than 100 cc which is composed of natural pulp alone or a mixture of natural pulp and synthetic pulp. The paper thus prepared is moistened so as to have a moisture content within the range of 5 to 30% and then subjected to a calendering treatment with the use of a heated embossing metal roll to transparentize the moistened paper and form a finely embossed surface thereon. The embossing metal roll has a peripheral surface engraved so as to have a surface roughness of a  $R_{max}$  of 20 to 200 microns and a relief peak number of 1 to 20 per 1 mm.

**BRIEF DESCRIPTION OF THE INVENTION**

FIG. 1 shows a chart whose vertical and horizontal magnifications are 1600 and 20, respectively, which is obtained by a measurement of the surface roughness of #800 embossing roll which was used in Examples. The measurement was carried out according to JIS BO601-1970 and JIS BO651-1970 with the use of a stylus having a radius of curvature of 5 microns at stylus head and with the use of a surface roughness tester SE-4 manufactured by Kosaka Laboratory, Ltd., Japan, and the results were recorded with aid of a self-balancing mono pen type recorder QPD-53 manufactured by Hitachi, Ltd., Japan, in which the available width of recording paper was 250 mm and the balancing rate was less than one second/full scale.

FIG. 2 shows a chart obtained by a measurement of the surface roughness of #400 embossing roll which was used in Examples. The measurement was carried out in the same manner as the above.

FIG. 3 shows a chart obtained in the same manner as the above with respect to the #300 embossing roll which was used in Examples of the invention, provided that the vertical magnification is 600.

FIG. 4 shows a chart obtained in the same manner as the above with respect to a conventional 46 mesh emery sand blast roll which was used in Controls.

FIG. 5 shows a chart obtained in the same manner as the above with respect to a matter transparent paper obtained in Example 1.

FIG. 6 shows a chart obtained in the same manner as the above with respect to a matted transparent paper obtained in Control 1.

FIG. 7 shows a chart obtained in the same manner as the above with respect to a matted transparent paper obtained in Example 3-1.

FIG. 8 shows a chart obtained in the same manner as the above with respect to a matted transparent paper obtained in Control 2-1.

FIG. 9 is a photograph of 50 magnifications showing a replica of the surface of #800 embossing roll which was used in Examples of the invention taken with an Electron Probe Microanalyzer, JXA-50A, manufactured by Japan Electron Optics Laboratory Co., Ltd.

FIG. 10 shows a photograph obtained in the same manner as the above with respect to #400 embossing roll which was used in Examples of the invention.

FIG. 11 shows a photograph obtained in the same manner as the above with respect to #300 embossing roll used in Examples of the invention.

FIG. 12 shows a photograph obtained in the same manner as the above with respect to 46 mesh emery sand blast roll which was used in Controls.

FIG. 13 is a schematic elevational view of a super calender used in Example 1.

FIG. 14 is a schematic elevational view of a super calender used in Example 3.

30

35

40

45

50

55

60

65

range of 100:0 to 10:90. It is not desirable to use the synthetic pulp alone for making a paper because the paper prepared from synthetic pulp alone changes into a film by heat and pressure of this invention.

The conventional additives such as sizing agents; fixing agents; releasing agents; fillers; dyestuffs; adhesives such as starch, polyvinyl alcohol, carboxy methyl cellulose, sodium alginate and aqueous solutions or emulsions of synthetic resins or polymers; transparentizing agents; transparentizing assistants; and antistatic agents may be used in the process of paper making.

A paper prepared from the pulp suspension having the beating degree described above with the use of a conventional paper machine such as a Fourdrinier paper machine and a cylinder paper machine has various difficulties in the transparentization of paper. The lightly beaten pulp much differs in its fiber structure from the heavily beaten pulp. In case of lightly beaten natural pulp, the fibers are not so much injured but remain a rigid spindle form and accordingly a number of intercellular spaces remain in the fibers. Therefore, the paper prepared from such natural pulp shows a high resistivity against transparentization by an application of heat and pressure. Similarly, the lightly beaten synthetic pulp has a rigid rod-like spindle or random structure which gives a high resistivity against transparentization. Furthermore, such a lightly beaten pulp forms a loose paper layer because the lightly beaten pulp fibers have a relatively large diameter, for example, within the range of 10 to 30 microns and a relatively long fiber length, for example, within the range of 1 to 3 mm, which raises difficulties in transparentizing by the application of moisture, heat and pressure. Since the lightly beaten pulp is superior in a drainage in a wire part of paper machine to the heavily beaten pulp, a paper making rate is increased. However, the lightly beaten pulp additionally tends to give wire marks on the surface of the resultant paper which cause an undesirable effect on the uniform transparentization of the resultant paper together with other factors such as felt marks formed in a press part and wrinkles and cocklings formed in a dryer part which concern with the surface structure of paper.

According to the invention, the above mentioned disadvantages inherent in the use of such a lightly beaten pulp can be avoided by utilizing a special embossing metal roll.

As the embossing metal roll of the invention, there may be used a metal roll having such a finely rugged surface that  $R_{max}$  is within the range of 20 to 200 microns, preferably 25 to 160 microns, and a relief peak number is within the range of 1 to 20 per 1 mm, preferably 2 to 15 per 1 mm. A definition of the term of  $R_{max}$  is as follows. According to JIS BO601-1970 and JIS BO 651-1970, the roll surface is scanned with a stylus having a radius of curvature of 5 microns at the stylus head of under the conditions of a stylus pressure of 0.4 g and a scanning velocity of 0.2 mm/sec. to obtain a chart. A straight line which contacts with three peaks with exception of the highest peak on the thus obtained chart is drawn as a standard line. A distance from the standard line to the deepest bottom of the curve which exists in a region to which the standard line belongs is defined as  $R_{max}$ . When the value of  $R_{max}$  is out of the range defined herein, a paper having a good balance of quality cannot be obtained. In addition, it is not preferable to use such a roll whose  $R_{max}$  is beyond the range defined in the present invention because it is liable to injure an

#### DETAILED DESCRIPTION OF THE INVENTION

In this invention, it is an essential requirement that the paper used in the invention should be prepared from an aqueous suspension of pulp whose beating degree is larger than 100 cc in CSF and which contains natural pulp alone or a mixture of natural pulp and synthetic pulp. The term of beating degree means that of the pulp suspension in the prior state to paper making. Among the pulp suspension there are included a suspension of beaten virgin pulp, a suspension of disintegrated pulp from waste papers and a mixture thereof. In addition, even if pulp itself has a beating degree out of the range defined in the invention, it may be used provided that the beating degree falls within the range defined upon mixing it with other pulp.

Among the pulp suspensions having beating degree of the specific range described above, that having the beating degree of 150 to 650 cc in CSF is preferable and that having the beating degree of 200 to 600 cc in CSF is the most preferable.

As natural pulp, any kind of natural pulp available for a wet paper making such as wood pulp and the other natural pulp, for example, those prepared from bast fibers, animal fibers and the like may be used. Among them the wood pulp is the most preferable.

As synthetic pulp, any kind of synthetic pulp available for a wet paper making process may be used. For example, such a synthetic pulp is disclosed in Japanese Patent Publications No. 8,565 of 1960, No. 19,602 of 1963, No. 2,302 of 1964, No. 10,183 of 1968 and No. 32,458 of 1971, Japanese Laid-Open Patent Publications No. 35,319 of 1972, No. 35,225 of 1972, No. 29,820 of 1975, No. 36,731 of 1975 and No. 40,803 of 1975. In this invention, the synthetic pulp is used in the form of a mixture with natural pulp. The mixture ratio by weight of natural pulp to synthetic pulp should be within the

elastic roll which is used in combination with the embossing roll in order to form a nip.

The term of "relief peak number" refers to the number of peaks per 1 mm of scanning distance on the same chart obtained in the above mentioned measurement of Rmax. Upon the calculation of the relief peak number, extremely low peaks, i.e., those having a height less than 5% of Rmax, should be neglected. Each of Rmax and the relief peak number represents an arithmetic means value of randomly selected respective ten results of 10 measurements. Each of the relief peaks may preferably be sharp. When the value of the relief peak number is out of the range of 1 to 20 per 1 mm, it would be impossible to obtain a paper having a uniform transparency and a desired surface roughness.

Among methods for manufacturing the above mentioned embossing roll, an engraving method in which the patterns engraved on a mother roll are reproduced on the surface of the metal roll is the most preferable. The particular unenven surface structures may contribute to enhancing a microscopic linear pressure effect of the roll, a heat transfer effect and a removing effect of air and moisture from the paper layer. Therefore, a uniform transparency can be obtained even on such a paper that has a large interfibrous space therein or an appreciable wire mark or that is inferior in a thermoplasticity.

On the contrary, when an embossing metal roll prepared by a conventional sand blast method is used, the pressure may be applied to the paper rather in a state of surface pressure from a microscopic viewpoint and accordingly the pressure may not be sufficiently applied to such a part of the paper in which the interfibrous spaces and the wire marks exist. Consequently, a uniform transparency cannot be obtained. The resultant paper has a number of misty opaque spots.

This invention does not intend to limit the material for the embossing metal roll; but metal roll made of cast iron, alloys including nickel and/or chrome, or steel and rolls whose surface is plated with hard chrome are preferably used. The embossing metal roll may also be provided with an internal heating or cooling device therein.

In the present invention, a good matted paper may be obtained even when the moisture content of the paper upon passing through a nip of the embossing metal roll is relatively low, i.e., within the range of 5 to 30%, preferably 7 to 27%. Generally, the moisture contained in paper serves as a plasticizer for pulp, a heat transfer medium, or a remover of air contained in the paper to make speedily it transparent. However, according to the invention, it is possible to attain a sufficient transparentization even when the moisture content is relatively low because the particular embossing metal roll of the invention contributes immensely to enhancing the transparentization. Especially, when a synthetic pulp is used for making a paper, the desired results may be obtained in a lower region of moisture content of the paper because the synthetic pulp is mainly composed of thermoplastic polymer and has an extremely low content of equilibrium moisture. As a method for moistening the paper until the moisture content falls within the range described hereinbefore, there may be used a conventional moistening method such as a coating method with use of a conventional coating means, a spraying method and an electrostatic moistening method. In the process of moistening paper, the various additives such as sizing

agents, releasing agents, antistatic agents, transparentizing agents and dyestuffs may be added into water.

In the industrial practice of the invention, the embossing metal roll is used for the treatment of the paper in an embossing or calendering system. Fundamentally, a single nip emboss of machine consisting an embossing metal roll and an elastic roll which are contact under pressure to each other may be used. In case of a multistack super calendering system having a plurality of nips at least one of chilled rolls may be replaced by the embossing metal roll according to the invention. This invention does not intend to limit the material for the elastic roll and its hardness, but cotton, paper, asbestos, synthetic fibers for fiber roll and hard rubber are desirably used as a material. Referring to the hardness of the elastic roll, one having a shore hardness not less than 70° is preferable.

The temperature of the embossing metal roll should not be limited to a specific range but is determined 20 depending upon the various factors such as moisture content, pulp composition, weight of paper and number of nip. When a multiplicity of the embossing rolls is used, each roll may be at the different temperatures. However, it may be generally within the range of 50° to 25 200° C., preferably 80° to 180° C.

The pressure to be applied on the paper is not limited as well. In case of treating a paper comprising synthetic pulp having a low softening point, the pressure may be relatively low. When the paper comprises a large quantity of natural pulp, a relatively high pressure is preferably applied. Generally, the pressure may be controlled within the range of 20 to 600 kg/cm, preferably 40 to 400 kg/cm.

The matted paper obtained according to the invention has a uniform transparency without any misty opaque spot inherent in the use of lightly beaten pulp and has an excellent writability. In addition, since a paper prepared from lightly beaten pulp is used as a base sheet in the invention, the resultant matted paper has an 45 excellent dimensional stability to moisture or water and accordingly it further has an excellent secondary processability, for example, an excellent printability, printing workability in offset printing and coating workability of an aqueous coating composition compared with a conventional transparent paper. The matted paper of the invention is suitable for various base papers such as a base paper for pressure sensitive copying paper, releasing paper and etc.

The invention will be further illustrated by reference 50 to the following examples, however, the invention is not limited to those examples but includes wide variations.

Unless otherwise indicated, parts and % signify parts by weight and % by weight, respectively.

#### EXAMPLE 1

A paper was made from a pulp suspension having a CSF of 400 cc prepared from 20 parts of a bleached needle-leaved kraft pulp (N) having a CSF of 380 cc and 80 parts of a bleached broad-leaved kraft pulp (L) having a CSF of 450 cc with the use of a Fourdrinier paper machine. The moisture content of the resultant paper was adjusted to 23% by applying water to the sheet with a spray nozzle moistner. Then the sheet was passed through a fourteen stacks super calender in such a manner as shown in FIG. 13 so that both surfaces of the sheet might be subjected to the treatment with the embossing roll for two times. In FIG. 13 the fourteen

stacks super calender was provided with two embossing rolls (23,26) plated with hard chromium and having a surface engraved so as to have  $R_{max}$  of 34.3 microns and a relief peak number of 8 per 1 mm (hereinafter referred to as #800 embossing roll) at the third and sixth position from the bottom and also having conventional chilled rolls (21, 28, 30, 32, 34) and elastic rolls (22, 24, 25, 27, 29, 31, 33). The surface temperatures of the third roll (23) and sixth roll(26) were 155° C. and 145° C., respectively. The maximum linear pressure of the final nip (35) was 220 kg/cm and the passing velocity of the paper was 50 m/min.

#### CONTROL 1

Example 1 was repeated except that the two #800 embossing rolls were replaced with two chilled rolls having smooth surfaces.

The properties of the papers obtained in Example 1 and Control 1 are shown in Table 1, FIG. 5 and FIG. 6. The matted transparent paper obtained in Example 1 had a high transparency and a good writability in pencil writing. The misty opaque spot was hardly appreciated. On the contrary, the transparent paper obtained in Control 1 was inferior in a transparency and the surface of the paper was too smooth to give a good writability at a normal writing pressure. In addition, a number of misty opaque spots in the form of wire marks formed on the surface of the base sheet during the paper making process were remarkably appreciated.

#### EXAMPLE 2

A synthetic pulp ( $S_1$ ) having a CSF of 250 cc was prepared by beating synthetic fibers having 7 denier, a length of 10 mm and a polyvinyl alcohol content of 10% which were obtained by wet spinning from a mixture of a polyvinyl alcohol (hereinafter referred to as PVA), acrylonitrile (hereinafter referred to as AN) graft copolymer in which a weight ratio of PVA/AN was 50/50 with an acrylonitril-styrene copolymer in which a weight ratio of AN/styrene was 24/76. Thus obtained synthetic pulp ( $S_1$ ), a bleached needle-leaved kraft pulp (N) having a CSF of 380 cc and a bleached broad-leaved kraft pulp (L) having a CSF of 450 cc (both used in Example 1) were mixed in the proportions shown in Table 2 and formed into papers in the same manner as in Example 1.

The moisture contents of the resultant papers were adjusted at 22% and then the papers were passed through the same super calender as in Example 1 in the same manner as in Example 1 except that the velocity of passing paper was 80 m/min to obtain matted transparent papers. The properties of the resultant matted transparent papers are shown in Table 2. The matted transparent papers obtained in Example 2 were superior in transparency, writability in pencil writing, dimensional stability, paper strength and appearance.

#### EXAMPLE 3

The same synthetic pulp ( $S_1$ ) as used in Example 2, a bleached needle-leaved kraft pulp ( $N_1$ ) having a CSF of 580 cc and a bleached broad-leaved kraft pulp ( $L_1$ ) having a CSF of 620 cc were mixed in the ratio shown in Table 3 and formed into papers with a commercial paper machine. The moisture content of the resultant paper was adjusted at the value shown in Table 3.

Then the sheet was passed through a fourteen stacks super calender in such a manner as shown in FIG. 14 so that one side surface of the paper might be subjected to

the treatment with the embossing roll for four times and the reverse side surface of the paper might be subjected to the treatment with the embossing roll for one time.

In FIG. 14 the fourteen stacks super calender is the same one as in Example 1 except that the chilled roll having a smooth surface at the 8th position from the bottom was further replaced with an embossing roll (28) plated with hard chromium and having an engraved surface whose  $R_{max}$  was 53.7 microns and the relief peak number was 4 per 1 mm (hereinafter referred to as #400 embossing roll). The above treatment was carried out under the conditions that the highest temperature of the embossing roll was at 150° C., the maximum linear pressure of the final nip (35) was 240 kg/cm and the velocity of passing paper was 65 m/min. The properties of the resultant matted transparent papers are shown in Table 3.

#### CONTROL 2

Two kinds of moistened papers of Example 3-1 and 3-3 were subjected to the same treatment as in Example 3 except that the #400 embossing roll at the 8th position and the #800 embossing roll at the 6th position were replaced with two chilled rolls having smooth surfaces, respectively, and that the #800 embossing roll at the third position was further replaced with a 46 mesh emery sand blast roll plated with hard chromium and having a surface whose  $R_{max}$  of 11 microns and the relief peak number of 8 per 1 mm to obtain two kinds of transparent papers of Control 2-1 and 2-2, respectively. In this Control, only one side surface of the paper was treated with the 46 mesh emery sand blast roll. The properties of the thus obtained transparent papers are shown in Table 4. The transparent papers obtained in Control 2 were inferior to those obtained in Example 3 in the respects of a transparency and a writability in pencil writing. In addition, a number of misty opaque spots were appreciated.

#### EXAMPLE 4

A fibrous material ( $S_2$ ) having a CSF of 280 cc was prepared by beating the commercially available synthetic pulp prepared from poly-olefin (SWP: Product of Mitsui Zellerbach Co., Ltd.) with use of a Sprout-Waldron type single disk refiner under the conditions of the concentration of pulp at 3% and the clearance at 50 microns. Thus obtained fibrous material ( $S_2$ ), a bleached needle-leaved kraft pulp ( $N_2$ ) having a CSF of 450 cc and a bleached broad-leaved kraft pulp ( $L_2$ ) having a CSF of 500 cc were mixed in the ratio shown in Table 5 and formed into a paper with a manual paper-making sheet machine manufactured by Toyo Seiki, Co. Ltd.

The moisture content of the resultant sheet was adjusted at the value shown in Table 5. Then, the sheet was passed through a two stack test embossing machine manufactured by Yuri Roll Co., Ltd. which was provided with #800' embossing roll of smaller diameter than that of the #800 embossing roll used in the above Examples having the same engraved patterns as those of the above described #800 embossing roll and provided with an elastic roll under the conditions of the surface temperature of #800' embossing roll at 150° C. and the linear pressure at 200 kg/cm for four times in all, reversing the sheet upside-down.

#### CONTROL 3

The same treatment as in Example 4 was repeated with use of the same moistened sheet as in Example 4-2

except that the #800' embossing roll was replaced with a 46 mesh emery sand blast roll.

In Example 4, there was no trouble during the process of the treatment and the obtained transparent papers were superior in transparency, writability and appearance.

On the contrary, it was observed in Control 3 that the blisters were produced during the first treating process in which the paper had a high moisture content, owing to the so much minutely uneven surface of 46 mesh sand blast roll. The surface of the transparent paper obtained in Control 3 was not sufficiently matted and accordingly a good writability could not be attained. In addition, a large number of misty opaque spots were appreciated.

#### EXAMPLE 5

Synthetic pulp ( $S_3$ ) having a CSF of 350 cc was prepared by beating synthetic fibers having a PVA content of 20%, 1.2 denier and a length of 6 mm which were made by a wet spinning process from a mixture of a PVA-AN graft copolymer in which the weight ratio of PVA/AN was 50/50 with an AN-methylacrylate copolymer comprising 95 mol% of AN and 5 mol% of methyl acrylate.

The bleached needle-leaved kraft pulp ( $N_2$ ) having a CSF of 450 cc and the bleached broad-leaved kraft pulp ( $L_2$ ) having a CSF of 500 cc used in Example 4 were mixed with the above obtained synthetic pulp ( $S_3$ ) in the proportions shown in Table 6 and formed into papers by the same manual paper-making sheet machine as used in Example 4. The moisture content of the obtained papers was adjusted at the value shown in Table 6. Then, the papers were passed through a two stack test embossing machine (manufactured by Yuri Roll Co., Ltd.) provided with the #400 embossing roll and an elastic roll under the conditions of the temperature of the embossing roll at 160° C. and the linear pressure at 220 kg/cm for two times in all, reversing the paper upside-down. The properties of the obtained matted transparent pa-

10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755  
8760  
8765  
8770  
8775  
8780  
8785  
8790  
8795  
8800  
8805  
8810  
8815  
8820  
8825  
8830  
8835  
8840  
8845  
8850  
8855  
8860  
8865  
8870  
8875  
8880  
8885  
8890  
8895  
8900  
8905  
8910  
8915  
8920  
8925  
8930  
8935  
8940  
8945  
8950  
8955  
8960  
8965  
8970  
8975  
8980  
8985  
8990  
8995  
9000  
9005  
9010  
9015  
9020  
9025  
9030  
903

TABLE 1-continued

## Example-1

| Properties of transparent paper |     |     |                                     |                                  |                |                                |                |                            |      |
|---------------------------------|-----|-----|-------------------------------------|----------------------------------|----------------|--------------------------------|----------------|----------------------------|------|
| Sheet forming                   |     |     | Moisture content after moistening % |                                  |                | Expansion in water             |                |                            |      |
| Pulp composition on dry basis   |     |     | CSF of mixed pulp                   | Weight of sheet g/m <sup>2</sup> | (on wet basis) | Bulk density g/cm <sup>3</sup> | Transparency % | Specific tear factor MD/CD | CD % |
| N %                             | L % | S % | pulp cc                             | sheet g/m <sup>2</sup>           |                |                                |                |                            |      |
| good                            |     |     |                                     |                                  |                |                                |                |                            |      |

Note:

<sup>1</sup>Transparency (%) = 100 - value of opacity by Hunter reflectometer (JIS P-8138).<sup>2</sup>Tear factor was determined according to JIS P-8116.<sup>3</sup>Expansion in water was measured with a Fenchel expansion meter after dipping the sheet in water at 20° C. for 5 minutes.

The above notes are applicable throughout all the  
Tables 1 to 8.

TABLE 2

## Example-2

| Properties of transparent paper |      |     |                                     |                                  |                |                                |                |                            |       |      |    |      |          |
|---------------------------------|------|-----|-------------------------------------|----------------------------------|----------------|--------------------------------|----------------|----------------------------|-------|------|----|------|----------|
| Sheet forming                   |      |     | Moisture content after moistening % |                                  |                | Expansion in water             |                |                            |       |      |    |      |          |
| Pulp composition on dry basis   |      |     | CSF of mixed pulp                   | Weight of sheet g/m <sup>2</sup> | (on wet basis) | Bulk density g/cm <sup>3</sup> | Transparency % | Specific tear factor MD/CD | CD %  |      |    |      |          |
| N %                             | L %  | S % | pulp cc                             | sheet g/m <sup>2</sup>           |                |                                |                |                            |       |      |    |      |          |
| Example 2-1                     | 17.5 | 75  | 7.5                                 | 390                              | 40             | 22                             | 1.05           | 68                         | 12/39 | 1.95 | 13 | good | very few |
| Example 2-2                     | 40   | 45  | 15                                  | 320                              | 40             | 22                             | 1.05           | 72                         | 42/40 | 1.77 | 16 | good | very few |
| Example 2-3                     | 30   | 46  | 24                                  | 310                              | 40             | 22                             | 1.05           | 74                         | 39/37 | 1.48 | 18 | good | very few |

TABLE 3

## Example-3

| Properties of transparent paper |                  |                  |                                     |                                  |                |                                |                |                            |       |      |    |      |     |
|---------------------------------|------------------|------------------|-------------------------------------|----------------------------------|----------------|--------------------------------|----------------|----------------------------|-------|------|----|------|-----|
| Sheet forming                   |                  |                  | Moisture content after moistening % |                                  |                | Expansion in water             |                |                            |       |      |    |      |     |
| Pulp composition on dry basis   |                  |                  | CSF of mixed pulp                   | Weight of sheet g/m <sup>2</sup> | (on wet basis) | Bulk density g/cm <sup>3</sup> | Transparency % | Specific tear factor MD/CD | CD %  |      |    |      |     |
| N <sub>1</sub> %                | L <sub>1</sub> % | S <sub>1</sub> % | pulp cc                             | sheet g/m <sup>2</sup>           |                |                                |                |                            |       |      |    |      |     |
| Example 3-1                     | 50               | 35               | 15                                  | 460                              | 60             | 20                             | 1.05           | 67                         | 42/41 | 1.66 | 16 | good | few |
| Example 3-2                     | 15               | 75               | 10                                  | 500                              | 64             | 22                             | 1.10           | 65                         | 39/38 | 1.70 | 16 | good | few |
| Example 3-3                     | 30               | 55               | 15                                  | 470                              | 70             | 23                             | 1.05           | 62                         | 43/41 | 1.34 | 16 | good | few |
| Example 3-4                     | 30               | 30               | 40                                  | 350                              | 60             | 15                             | 1.00           | 72                         | 35/34 | 1.20 | 17 | good | few |

TABLE 4

## Control-2

| Properties of transparent paper |           |                        |                                     |                                           |                                  |                                      |                                |                                          |                            |      |   |                |      |
|---------------------------------|-----------|------------------------|-------------------------------------|-------------------------------------------|----------------------------------|--------------------------------------|--------------------------------|------------------------------------------|----------------------------|------|---|----------------|------|
| Sheet forming                   |           |                        | Moisture content after moistening % |                                           |                                  | Expansion in water                   |                                |                                          |                            |      |   |                |      |
| Pulp composition on dry basis   |           |                        | Synthetic pulp                      | CSF of mixed pulp                         | Weight of sheet g/m <sup>2</sup> | (on wet basis)                       | Bulk density g/cm <sup>3</sup> | Transparency %                           | Specific tear factor MD/CD |      |   |                |      |
| NBK%<br>LBK%<br>%               | LBK%<br>% | Synthetic<br>pulp<br>% | CSF of<br>mixed<br>pulp<br>cc       | Weight<br>of<br>sheet<br>g/m <sup>2</sup> | (on wet<br>basis)                | Bulk<br>density<br>g/cm <sup>3</sup> | Trans-<br>parency<br>%         | Speci-<br>fic<br>tear<br>factor<br>MD/CD | CD<br>%                    |      |   |                |      |
| Control 2-1                     | 50        | 35                     | 15                                  | 460                                       | 60                               | 20                                   | 1.05                           | 62                                       | 41/41                      | 1.60 | 4 | too flat<br>to | many |

TABLE 4-continued

## Control-2

|             | Properties of transparent paper |            |                  |                      |                                   |                             |                                |                |                            |                         |                          |                        |
|-------------|---------------------------------|------------|------------------|----------------------|-----------------------------------|-----------------------------|--------------------------------|----------------|----------------------------|-------------------------|--------------------------|------------------------|
|             | Sheet forming                   |            |                  |                      | Moisture content after moistening |                             |                                |                | Expansion in water         |                         |                          |                        |
|             | Pulp composition on dry basis   |            |                  | CSF of mixed pulp    | Weight of sheet g/m <sup>2</sup>  | moistening % (on wet basis) | Bulk density g/cm <sup>3</sup> | Transparency % | Specific tear factor MD/CD | Expansion in water CD % | Surface roughness Rmax μ | Pencil writability     |
|             | NBK%<br>%                       | LBKP%<br>% | Synthetic pulp % | CSF of mixed pulp cc | Weight of sheet g/m <sup>2</sup>  | moistening % (on wet basis) | Bulk density g/cm <sup>3</sup> | Transparency % | Specific tear factor MD/CD | Expansion in water CD % | Surface roughness Rmax μ | Pencil writability     |
| Control 2-3 | 30                              | 55         | 15               | 500                  | 70                                | 23                          | 1.05                           | 56             | 43/42                      | 1.37                    | 4                        | too flat to write many |

TABLE 5

## Example-4

|             | Properties of transparent paper |                       |                       |                      |                                   |                             |                                |                |                            |                         |                          |                        |
|-------------|---------------------------------|-----------------------|-----------------------|----------------------|-----------------------------------|-----------------------------|--------------------------------|----------------|----------------------------|-------------------------|--------------------------|------------------------|
|             | Sheet forming                   |                       |                       |                      | Moisture content after moistening |                             |                                |                | Expansion in water         |                         |                          |                        |
|             | Pulp composition on dry basis   |                       |                       | CSF of mixed pulp    | Weight of sheet g/m <sup>2</sup>  | moistening % (on wet basis) | Bulk density g/cm <sup>3</sup> | Transparency % | Specific tear factor MD/CD | Expansion in water CD % | Surface roughness Rmax μ | Pencil writability     |
|             | N <sub>2</sub> %<br>%           | L <sub>2</sub> %<br>% | S <sub>2</sub> %<br>% | CSF of mixed pulp cc | Weight of sheet g/m <sup>2</sup>  | moistening % (on wet basis) | Bulk density g/cm <sup>3</sup> | Transparency % | Specific tear factor MD/CD | Expansion in water CD % | Surface roughness Rmax μ | Pencil writability     |
| Example 4-1 | 20                              | 60                    | 20                    | 415                  | 50                                | 18                          | 1.10                           | 58.0           | 40/39                      | 1.31                    | 17                       | good very few          |
| Example 4-2 | 40                              | 10                    | 50                    | 340                  | 50                                | 15                          | 0.98                           | 74.3           | 37/37                      | 0.75                    | 18                       | good very few          |
| Example 4-3 | 20                              | —                     | 80                    | 290                  | 50                                | 9                           | 0.85                           | 77.3           | 34/32                      | 0.40                    | 21                       | good very few          |
| Control-3   | 40                              | 10                    | 50                    | 340                  | 50                                | 15                          | 0.90                           | 72.1           | 38/37                      | 0.71                    | 23                       | too flat to write many |

TABLE 6

## Example-5

|             | Properties of transparent paper |                       |                       |                      |                                   |                             |                                |                |                            |                         |                          |                    |
|-------------|---------------------------------|-----------------------|-----------------------|----------------------|-----------------------------------|-----------------------------|--------------------------------|----------------|----------------------------|-------------------------|--------------------------|--------------------|
|             | Sheet forming                   |                       |                       |                      | Moisture content after moistening |                             |                                |                | Expansion in water         |                         |                          |                    |
|             | Pulp composition on dry basis   |                       |                       | CSF of mixed pulp    | Weight of sheet g/m <sup>2</sup>  | moistening % (on wet basis) | Bulk density g/cm <sup>3</sup> | Transparency % | Specific tear factor MD/CD | Expansion in water CD % | Surface roughness Rmax μ | Pencil writability |
|             | N <sub>2</sub> %<br>%           | L <sub>2</sub> %<br>% | S <sub>3</sub> %<br>% | CSF of mixed pulp cc | Weight of sheet g/m <sup>2</sup>  | moistening % (on wet basis) | Bulk density g/cm <sup>3</sup> | Transparency % | Specific tear factor MD/CD | Expansion in water CD % | Surface roughness Rmax μ | Pencil writability |
| Example 5-1 | 30                              | 30                    | 40                    | 390                  | 60                                | 14                          | 0.95                           | 62.0           | 39/36                      | 0.90                    | 20                       | good very few      |
| Example 5-2 | 20                              | —                     | 80                    | 340                  | 60                                | 10                          | 0.88                           | 71.4           | 35/35                      | 0.52                    | 24                       | good very few      |

TABLE 7

## Control-4

|             | Properties of transparent paper |            |                  |                      |                                   |                             |                                |                |                            |                         |                          |                                  |
|-------------|---------------------------------|------------|------------------|----------------------|-----------------------------------|-----------------------------|--------------------------------|----------------|----------------------------|-------------------------|--------------------------|----------------------------------|
|             | Sheet forming                   |            |                  |                      | Moisture content after moistening |                             |                                |                | Expansion in water         |                         |                          |                                  |
|             | Pulp composition on dry basis   |            |                  | CSF of mixed pulp    | Weight of sheet g/m <sup>2</sup>  | moistening % (on wet basis) | Bulk density g/cm <sup>3</sup> | Transparency % | Specific tear factor MD/CD | Expansion in water CD % | Surface roughness Rmax μ | Pencil writability               |
|             | N <sub>3</sub> %<br>%           | LBKP%<br>% | Synthetic pulp % | CSF of mixed pulp cc | Weight of sheet g/m <sup>2</sup>  | moistening % (on wet basis) | Bulk density g/cm <sup>3</sup> | Transparency % | Specific tear factor MD/CD | Expansion in water CD % | Surface roughness Rmax μ | Pencil writability               |
| Control 4-1 | 100                             | —          | —                | 50                   | 30                                | 10                          | 0.95                           | 53.5           | 42/40                      | 4.25                    | 8                        | too flat to write relatively few |
| Control 4-2 | 100                             | —          | —                | 50                   | 50                                | 12                          | 1.03                           | 58.7           | 38/37                      | 4.34                    | 4                        | too flat to write relatively few |

TABLE 7-continued

Control-4

|             | Properties of transparent paper |        |                  |                      |                                     |                                                    |                                |                |                              |                         |                              |                   |                         |  |                              |  |                    |                    |
|-------------|---------------------------------|--------|------------------|----------------------|-------------------------------------|----------------------------------------------------|--------------------------------|----------------|------------------------------|-------------------------|------------------------------|-------------------|-------------------------|--|------------------------------|--|--------------------|--------------------|
|             | Sheet forming                   |        |                  |                      | Moisture content after moistening % |                                                    |                                |                |                              |                         |                              |                   | Expansion in water CD % |  | Surface roughness Rmax $\mu$ |  | Pencil writability | Misty opaque spots |
|             | Pulp composition on dry basis   |        | Synthetic pulp % | CSF of mixed pulp cc | Weight of sheet g/m <sup>2</sup>    | Moisture content after moistening % (on wet basis) | Bulk density g/cm <sup>3</sup> | Transparency % | Speci- fic tear factor MD/CD | Expansion in water CD % | Surface roughness Rmax $\mu$ |                   |                         |  |                              |  |                    |                    |
|             | N <sub>3</sub> %                | LBKP % | Synthetic pulp % | CSF of mixed pulp cc | Weight of sheet g/m <sup>2</sup>    | Moisture content after moistening % (on wet basis) | Bulk density g/cm <sup>3</sup> | Transparency % | Speci- fic tear factor MD/CD | Expansion in water CD % | Surface roughness Rmax $\mu$ |                   |                         |  |                              |  |                    |                    |
| Control 4-3 | 100                             | —      | —                | 50                   | 50                                  | 16                                                 | 1.12                           | 60.5           | 33/32                        | 4.26                    | 3                            | too flat to write | relatively few          |  |                              |  |                    |                    |

TABLE 8

Example-7

|             | Properties of transparent paper |                  |                                    |                      |                                           |                                           |                                            |                                |                      |                        |                      |                              |                              |      |                    |                    |
|-------------|---------------------------------|------------------|------------------------------------|----------------------|-------------------------------------------|-------------------------------------------|--------------------------------------------|--------------------------------|----------------------|------------------------|----------------------|------------------------------|------------------------------|------|--------------------|--------------------|
|             | Sheet forming                   |                  |                                    |                      | Moisture content after first moistening % |                                           | Moisture content after second moistening % |                                | Expansion in water % |                        |                      |                              | Surface roughness Rmax $\mu$ |      | Pencil writability | Misty opaque spots |
|             | Pulp composition on dry basis   |                  | S <sub>4</sub> or S <sub>5</sub> % | CSF of mixed pulp cc | Weight of sheet g/m <sup>2</sup>          | Moisture content after first moistening % | Moisture content after second moistening % | Bulk density g/cm <sup>3</sup> | Transparency %       | Speci- fic tear factor | Expansion in water % | Surface roughness Rmax $\mu$ |                              |      |                    |                    |
|             | N <sub>2</sub> %                | L <sub>2</sub> % | S <sub>5</sub> %                   | CSF of mixed pulp cc | Weight of sheet g/m <sup>2</sup>          | Moisture content after first moistening % | Moisture content after second moistening % | Bulk density g/cm <sup>3</sup> | Transparency %       | Speci- fic tear factor | Expansion in water % | Surface roughness Rmax $\mu$ |                              |      |                    |                    |
| Example 6-1 | 35                              | 45               | S <sub>4</sub>                     | 20                   | 520                                       | 50                                        | 17                                         | 14                             | 1.12                 | 66                     | 43                   | 0.81                         | 12                           | good | few                |                    |
| Example 6-2 | 35                              | 25               | S <sub>4</sub>                     | 40                   | 565                                       | 50                                        | 16                                         | 13                             | 1.10                 | 73                     | 38                   | 0.52                         | 13                           | good | few                |                    |
| Example 6-3 | 35                              | 45               | S <sub>5</sub>                     | 20                   | 515                                       | 50                                        | 17                                         | 14                             | 1.13                 | 65                     | 42                   | 0.76                         | 13                           | good | few                |                    |
| Example 6-4 | 35                              | 25               | S <sub>5</sub>                     | 40                   | 545                                       | 50                                        | 15                                         | 14                             | 1.07                 | 69                     | 37                   | 0.50                         | 14                           | good | few                |                    |

What we claim is:

1. A matted transparent paper manufactured by the steps of preparing a paper from an aqueous suspension of pulp having a CSF larger than 100 cc, moistening said paper so as to have a moisture content within the range of 5 to 30%, and calendering said moistened paper with the use of a heated embossing metal roll having a surface temperature of 50° to 200° C. to transparentize said moistened paper and form a finely embossed surface thereon, said embossing metal roll having a peripheral surface engraved so as to have a surface roughness of a Rmax of 25 to 160 microns and a relief peak number of 1 to 20 per 1 mm, and said pulp consisting essentially of wood pulp or a mixture of wood and synthetic pulp, at least 10% by-weight of the mixture being wood pulp.

2. A matted transparent paper as defined in claim 1, wherein said pulp has a CSF within the range of 150 to 650 cc.

3. A matted transparent paper as defined in claim 2, wherein said pulp has a CSF within the range of 200 to 600 cc.

4. A matted transparent paper as defined in claim 1, wherein said paper is moistened so as to have a moisture content within the range of 7 to 27%.

5. A matted transparent paper as defined in claim 1, wherein said relief peak number is within the range of 2 to 15 per 1 mm.

6. A matted transparent paper as defined in claim 1, wherein said moistened paper is calendered under pressure within the range of 20 to 600 kg/cm.

7. A matted transparent paper as defined in claim 6, wherein said moistened paper is calendered under pressure within the range of 40 to 400 kg/cm.

8. A matted transparent paper as defined in claim 1, wherein the surface temperature of said embossing metal roll is within the range of 80° to 180° C.

\* \* \* \* \*